

# UNITED STATES PATENT OFFICE.

CHARLES FELL, OF ELYRIA, OHIO, ASSIGNOR TO NATIONAL TUBE COMPANY, OF PITTSBURGH, PENNSYLVANIA, A CORPORATION OF NEW JERSEY.

## COATING MIXTURE.

1,358,304.

Specification of Letters Patent.

Patented Nov. 9, 1920.

No Drawing.

Application filed January 23, 1920. Serial No. 353,529.

To all whom it may concern:

Be it known that I, CHARLES FELL, a citizen of the United States, and resident of Elyria, in the county of Lorain and State of Ohio, have invented certain new and useful Improvements in Coating Mixtures, of which the following is a specification.

This invention relates to fluid coatings applied as a protective coating to prevent oxidation or rusting of metal surfaces and, while not limited to such use, more particularly relates to fluid coatings for metal pipes or tubes and is adapted to be applied after the pipes or tubes are completed, as a protective covering to the surface of welded pipes and tubes to prevent oxidation or rusting of the surfaces of the materials while in storage and during transportation from the place of manufacture to a place of use.

One object of my invention is the provision of a fluid coating of novel composition in which cheap and easily obtainable ingredients are employed.

Another object of the invention is to provide a protective coating which has sufficient fluidity to be applied in a rapid, cheap, and economical manner, and which is adapted to quickly dry on the coated metal surfaces after application.

A still further object of the invention is to provide a coating fluid of improved composition which has the required degree of fluidity and is adapted to be sprayed upon the surfaces being coated.

Still further objects will be made apparent as the invention becomes more fully described hereinafter.

My invention broadly consists in a novel composition composed of boiled linseed oil mixed with petroleum naphtha, and a mixture of hydrocarbon oils of the aromatic group and obtained by the destructive distillation of coal.

A specific example of such mixture, which has been proved to give very satisfactory results, is boiled linseed oil, petroleum naphtha, and a hydrocarbon oil containing benzol and its homologues such as toluo, xylol, etc. The materials and proportions used in making such composition are—

Boiled linseed oil—15 per cent.  
Petroleum naphtha—10 per cent.

Hydrocarbon oil of the aromatic group (containing benzol and its homologues)—75 per cent.

In all cases at least 50 per cent. of the benzol containing oil should be used in making the mixture, and in some cases it will be found of advantage to add about 3 per cent. of japan drier to the linseed oil, in making the composition. It is found that the amounts of the various materials used may be readily varied within the following proportions.

Boiled linseed oil (either with or without japan drier)-----12 to 18 per cent.  
Petroleum naphtha-----8 to 12 per cent.  
Hydrocarbon oil of the aromatic group and containing benzol and its homologues-----70 to 80 per cent.

In making the composition the japan drier, when used, will be added to and thoroughly mixed with the linseed oil. The petroleum naphtha will then be mixed with the linseed oil after which the hydrocarbon oil will be added to the mixture of linseed oil and naphtha. The hydrocarbon oil being a "thinner" will be added in quantities sufficient to give the fluidity required for spraying the mixture in applying it.

In applying the composition to metal surfaces such as pipes and tubes it preferably will be sprayed thereon, so as to cover the surfaces of the treated materials with a thin protective coating which, after becoming dry, effectively prevents rusting of the coated materials, even when exposed to the elements for long time intervals.

It is found when the mixture is applied the hydrocarbon oils and naphtha evaporate quickly and the linseed oil dries, leaving a residue which forms a thin, hard protective covering on the coated surfaces which effectively prevents rusting of the coated surfaces.

The advantages of my invention will be apparent to those skilled in the art. The various materials used in making my improved spraying mixture or composition of matter are readily obtained, are cheap and readily mix, while after being applied the mixture dries rapidly and forms a protection against rusting which is equal to or better than more expensive compositions used heretofore for that purpose.

I claim:

1. A metal surface protecting mixture consisting essentially of boiled linseed oil,

petroleum naphtha, and a hydrocarbon oil of the aromatic group.

2. A metal surface protecting mixture consisting essentially of boiled linseed oil, petroleum naphtha, and a hydrocarbon oil of the aromatic group containing benzol and its homologues.

3. A metal surface protecting mixture consisting essentially of from 12 to 18 per cent. linseed oil, from 8 to 12 per cent. petroleum naphtha, and from 70 to 80 per cent. of a hydrocarbon oil of the aromatic group.

4. A metal surface protecting mixture

consisting essentially of 15 per cent. lin- 15  
seed oil, 10 per cent. petroleum naphtha,  
and 75 per cent. of a hydrocarbon oil of the  
aromatic group.

5. A metal surface protecting mixture consisting of from 12 to 18 per cent. lin- 20  
seed oil, 3 per cent. japan drier, from 8 to  
12 per cent. petroleum naphtha, and from  
70 to 80 per cent. of a hydrocarbon oil of  
the aromatic group.

In testimony whereof, I have hereunto set 25  
my hand.

CHARLES FELL.